

## UNITED STATES PATENT OFFICE.

JOHN CHRISTOPHER MCGUIRE, OF DETROIT, MICHIGAN.

## STEEL.

No Drawing.

Application filed August 17, 1925. Serial No. 50,878.

This invention relates to manufacture of steel, its object being to provide a substitute for high speed steel of a composition particularly suitable for making cutting tools and dies and parts subjected to great abrasive wear by alloying together a mixture of a small quantity of tungsten, nickel and titanium with a high percentage chromium-carbon steel. I have made several tests 10 of various compositions of high chromium-carbon steels such as are manufactured to resist abrasive wear for such purposes as pulverizing machinery parts, burglar-proof safe plate, steam-shovel pins, dipper teeth etc. which because of its extreme hardness 15 also can be used for edge tools with far more efficiency than ordinary tool steel, and greatly improved by addition of a small amount of tungsten and will keep a very fine keen edge while cutting at high speeds. 20

Heretofore, standard grades of high speed steel which contain more or less of these same ingredients especially a high percentage of tungsten have been designed and 25 used for fast cutting and milling tools, etc. and its use is almost entirely limited to lathe, planer, boring, milling and similar cutters for rough machining operations and the work generally requires an additional machine operation, using high carbon tool steel cutters or special oil hardening steel cutters 30 to give the necessary fine smooth finish to the work and this must be done at a very low speed to preserve the keen edge on these 35 finishing cutters.

As a result of my experiments I have found that a good substitute for high speed steel can be made containing comparatively high percentages of carbon and chromium, 40 from  $2\frac{1}{4}$  percent to 8 percent tungsten and a small amount of nickel and titanium, this composition after casting or machining to desired shape also permits of the steel responding to hardening treatment at a considerably lower heat than is required for 45 high tungsten steels thereby preserving the fine edges and surface of intricate shaped tools, dies etc.

A steel according to my invention may be defined as containing from  $2\frac{1}{4}$  to 8 percent 50 of tungsten, from 0.90 to 3 percent carbon, from  $5\frac{1}{2}$  to 18 percent chromium, from 0.25 to 0.35 percent titanium, from 0.80 to 0.90 percent nickel.

A sample of the new steel according to 55 my invention shows the following analysis:

|            | Per cent. |
|------------|-----------|
| Carbon     | 1.40      |
| Tungsten   | 4.00 60   |
| Chromium   | 11.50     |
| Titanium   | .30       |
| Nickel     | .85       |
| Silicon    | .35       |
| Manganese  | .23 65    |
| Phosphorus | .025      |
| Sulphur    | .025      |
| Iron       | 81.32     |
|            | 100.00 70 |

Other metals may be added to steel of my present invention such as molybdenum, zirconium, uranium, vanadium, tantalum, up to about  $2\frac{1}{2}$  per cent that will vary the 75 properties somewhat but can be used to advantage for some purposes.

What I claim and desire to secure by Letters Patent is:—

1. A steel possessing substantially the following analysis:—Carbon 1.40 per cent, tungsten 4 per cent, chromium 11.50 per cent, titanium 0.30 per cent, nickel 0.85 per cent, silicon 0.35 per cent, manganese 0.23 per cent, phosphorus 0.025 per cent, sulphur 80 0.025 per cent, and iron 81.32 per cent, substantially as described.

2. A steel containing 2.25% to 8% of tungsten, 0.90 to 3% carbon, 7 to 18% chromium, 0.25 to 0.35% titanium, 0.80 to 0.90% nickel. 85

3. A steel of the composition of claim 2 plus not over about  $2\frac{1}{2}$  per cent of one of the following metals viz, molybdenum, zirconium, uranium, vanadium, tantalum.

JOHN CHRISTOPHER MCGUIRE.